

## UNITED STATES PATENT OFFICE

2,318,818

## PRODUCTION OF COLORED PHOTOGRAPHIC IMAGES

Alan Gilbert Tull, Purley, England, assignor to  
Latta Syndicate Limited, London, England, a  
British company

No Drawing. Application April 3, 1941, Serial No.  
386,744. In Great Britain April 4, 1940

8 Claims. (Cl. 95—2)

The present invention relates to the production of colored photographic images and it has for its principal object to provide a method of improving or modifying the characteristics of images produced by chemical toning processes, that is those in which the silver of a developed image or the residual halide after such development, is converted directly or indirectly to a metallic salt or compound, in general a colored salt.

In my co-pending application Serial No. 378,301, filed February 10, 1941, a method of producing reversed chemically toned images from the residual halide of a silver halide emulsion is described in which a silver ferrocyanide is first produced which is converted to various metal salt images such as Prussian blue or uranium ferrocyanide. In my co-pending application Serial No. 378,302, filed February 10, 1941, a process of producing multi-color records by producing chemically toned images at different depths of a silver halide emulsion layer or layers is described in which a Prussian blue image is formed in a surface layer or stratum while there is a red image of a uranium ferrocyanide below that. In my co-pending application Serial No. 384,180 filed March 19, 1941, the production of a three color record is described in which a uranium ferrocyanide image is formed in a middle layer. In all these processes it may be found that a chemically toned image has not the desired spectral absorptions or that the image obtained is not sufficiently permanent. Thus in the particular case of a uranium ferrocyanide image, the color of the image is not altogether satisfactory if the image is to form the magenta component of the three color picture while, as described in said co-pending application Serial No. 384,180 it may in some cases be desired to have a yellow image in that layer, and a more specific object of the invention is to modify or improve the color of such a uranium ferrocyanide image to render it more suitable as the red, or more correctly magenta, image of the three color picture, although the invention is equally applicable to the red image of a two color picture. A further object of the invention is to enable a yellow image to be produced in the layer in which the uranium ferrocyanide image is first formed. The present invention also enables the color contrast of a colored image to be varied as explained hereinafter.

In accordance with the present invention a chemically toned image or a conversion product derived therefrom is toned in a dye toning bath containing a dye which gives the desired color

and which mordants to that image or said conversion product.

The present invention is applicable to a chemically toned image either forming a monochrome picture or forming one of the component color records of a multi-color photographic picture, and the invention will be first described as applied to the toning of a single color picture. It is assumed that as a result of the preceding processing there is in the layer a silver salt image which is preferably silver ferrocyanide or another metal salt image produced from said silver ferrocyanide by chemical toning processes. Some of said images have been found to be mordants for certain dyestuffs and accordingly one feature of the present invention consists in the dye-toning of such a metallic salt image directly with an appropriate dye which mordants thereto.

It has been found however that a wider choice of dyestuffs for dye-toning is possible if the mordant consists of zinc ferrocyanide or one of its double salts. Such zinc ferrocyanide may be produced directly from the silver ferrocyanide by treatment in a zinc salt solution or if the silver ferrocyanide has been preliminarily converted into some other metal ferrocyanide, treatment in a zinc salt solution will in general convert that salt into zinc ferrocyanide owing to the extremely low solubility thereof. This salt has been found to be a particularly efficient mordant for a large number of basic dyestuffs.

As explained in my said co-pending application Serial No. 378,302 multi-color pictures may be produced in multi-layer photographic material containing intermediate images such as silver ferrocyanide, by means of a mixed toning bath of which one of the components is preferably a ferric salt, producing an image of Prussian blue in the surface layer and another component is a uranium salt producing an image of uranium ferrocyanide below the Prussian blue image. A particularly important advantage of the present invention is that it enables said uranium ferrocyanide image to be partially or wholly converted into a dye-toned image which as explained in co-pending application Serial No. 384,180 may be either magenta or yellow according to the characteristics of the material. This aspect of the invention is based on the discovery that when images consisting of Prussian blue and uranium ferrocyanide are treated in a solution of a zinc salt, the Prussian blue image is substantially unaffected while the uranium ferrocyanide is converted into zinc ferrocyanide which may then be toned for instance with Rhodamine G (Rowe

color index No. 750) or Auramine O (Rowe color index No. 655) according to whether a magenta or yellow image is required.

As a specific example illustrating the present invention it will be assumed that an exposure has been made on to a material of the type described in co-pending application Serial No. 384,180 and that it is desired to process the material to form a natural color positive by reversal. After development of the latent images in a developer containing a silver solvent such as thiocyanate, the material is treated in a conversion bath as described in said co-pending application Serial No. 378,301 to produce in all layers reversed deposits of a silver ferrocyanide, after which the material is treated in a mixed toning bath as described in said co-pending application Serial No. 378,302 to form a Prussian blue image in the outer layer followed by a uranium ferrocyanide image in the middle layer; a colored image being formed in the lower layer by selective destruction of the diffused dyestuff therein at any suitable stage in the operations. The uranium ferrocyanide image may not be of the desired magenta color and/or it may be desired to modify the color contrast thereof and in accordance with the present invention the uranium ferrocyanide image in the middle layer is converted into zinc ferrocyanide by treating the material for instance in the following bath:

| Cc.                         |    |
|-----------------------------|----|
| Oxalic acid, 5%             | 5  |
| Zinc sulphate, 10% solution | 5  |
| Water to                    | 20 |

The material is then washed for 10 minutes and thereupon or at some later stage, treated in a suitable dye bath. For magenta such a dye bath may consist of Rhodamine G (Rowe color index No. 750) containing sufficient acetic acid to bring the strength of the latter to 1%. The material is then washed until the high lights are clear, acidulated water being used if necessary. If a yellow image should be desired in the middle layer Rhodamine may be replaced by Auramine O (Rowe color index No. 655).

The two baths could be combined into a single bath which both performs the conversion of the uranium ferrocyanide into zinc ferrocyanide and the dye-toning of the latter.

In the foregoing example the production of reversed images is assumed but the invention is also applicable to non-reversal processing in which a developed silver image is bleached to a silver salt image and a conversion product derived therefrom is treated in a dye toning bath.

It should be noted that the zinc sulphate conversion bath given above is without effect on the Prussian blue image in the top layer after the latter has been formed while, further, the dye baths given have no effect on the Prussian blue image, that is to say the dye does not become mordanted to the image deposit in that layer, enabling the color of the image in the under layer to be corrected without affecting the color in the top layer.

The procedure given herein enables a color positive or negative to be produced in a very simple manner and of satisfactory color properties.

I claim:

1. A method of producing a colored photographic image, which comprises producing a uranium ferrocyanide image; bathing said image in a zinc salt bath to form a zinc salt mordant

image by reaction with the uranium ferrocyanide; and dye toning with a dye which mordants to said mordant image.

2. A method of producing a colored photographic image, which comprises producing a uranium ferrocyanide image; treating said image in a solution containing a zinc salt and oxalic acid to form a zinc salt mordant image by reaction with the uranium ferrocyanide; and dye toning said mordant image in a bath containing a dye which mordants to said mordant image.

3. A method of producing a colored photographic image, which comprises producing a uranium ferrocyanide image; and treating said image in a bath containing a zinc salt which is capable of producing a zinc salt mordant image by reaction with the uranium ferrocyanide, and a dye capable of being mordanted to said mordant image.

4. A method of producing multi-color photographic images in a multi-layer photographic material, which comprises the steps of producing chemically toned images in at least some of said layers, of which one image consists of uranium ferrocyanide; bathing the material in a solution containing a zinc salt to form a mordant image from said uranium ferrocyanide, the images present in the other layers being such as to be unaffected by said zinc salt bath; and dye toning with a bath containing a dye capable of mordanting to said mordant image.

5. A method of producing multi-color photographic images in a multi-layer photographic material, comprising forming silver ferrocyanide images in said layers, treating in a mixed toning bath containing a ferric salt and a uranium salt to form a Prussian blue image in the outer layer and a uranium ferrocyanide image in the following layer, treating in a zinc salt bath to convert the uranium ferrocyanide into a zinc salt mordant and dye toning the said mordant.

6. A method of producing multi-color photographic images in a photographic material having three superimposed photographic silver halide layers comprising producing silver ferrocyanide images in said layers surrounded by a complementary deposit unaffected by the further processing, treating in a mixed toning bath containing a ferric salt and a uranium salt to form a Prussian blue image in the surface layer and a uranium ferrocyanide image in the following layer, treating in a zinc salt bath to convert the uranium ferrocyanide into a zinc salt mordant, dye toning the latter and at any appropriate stage forming a color image in the third layer.

7. A method of producing multi-color photographic images in a photographic material having three superimposed photographic silver halide layers comprising exposing such material to produce latent images in the three layers, developing such latent images, converting the residual halide in such layers in a solution containing a conversion reagent and a complex-forming substance to form a silver ferrocyanide, treating the material in a mixed toning bath containing a ferric salt and a uranium salt to form a Prussian blue image in the surface layer and a uranium ferrocyanide image in the following layer, converting the uranium ferrocyanide image into a zinc salt mordant, dye toning the latter and at any appropriate stage producing a color image in the third layer.

8. A method of producing multi-color photographic images in a photographic material having three superimposed photographic silver hal-

ide layers comprising exposing such material to produce latent images in the three layers, developing such latent images, converting the developed images into silver ferrocyanide, treating the material in a mixed toning bath containing a ferric salt and a uranium salt to form a Prussian blue image in the surface layer and a uranium

ferrocyanide image in the following layer, converting the uranium ferrocyanide image into a zinc salt mordant, dye toning the latter and at any appropriate stage producing a color image in the third layer.

5 ALAN GILBERT TULL.